

Jan. 9, 1940.

F. D. WIDNER

**2,186,690**

## METHOD OF PRODUCING A CARBURIZING GAS

Filed July 8, 1937



Inventor  
*F. D. Widner*

34

Charles A. Lind  
Attorney

## UNITED STATES PATENT OFFICE

2,186,690

## METHOD OF PRODUCING A CARBURIZING GAS

Franklin D. Widner, Toledo, Ohio, assignor to  
Surface Combustion Corporation, Toledo,  
Ohio, a corporation of New York

Application July 8, 1937, Serial No. 152,626

3 Claims. (Cl. 148—17)

This invention relates to the art of carburizing steel articles to make them resistant to wear.

It is known that the articles may be carburized by exposing them while in a heated condition to 5 a gaseous atmosphere comprising a mixture of charcoal gas and natural gas.

In districts where natural gas is not available, it is customary to use bottled gases, such as, propane and butane, for enriching the charcoal gas. 10 However, when a hydrocarbon gas other than pure natural gas is simply added to the charcoal gas, it invariably happens that when the articles are removed from the carburizing retort, they will be found to be coated with a tightly adhering 15 scale having the appearance of an oxide scale but which on analysis is found to be a hard and dense coating of coke-like material which is metallic in appearance. Such coating interferes with normal carburization and frequently prevents it entirely.

The object of the present invention is to provide an improved method of utilizing the higher hydrocarbons and more particularly commercial propane and butane for enriching charcoal gas 25 in such a way that articles may be carburized without the formation of the objectionable coating above referred to.

In accordance with the present invention, the charcoal gas is enriched by flowing a stream of 30 hydrocarbon gas into the incandescent charcoal of a charcoal gas producer. By thus enriching the charcoal gas, it may be utilized without any further treatment as a carburizing gas and articles carburized in such a gas will be devoid of the 35 objectionable coating above referred to.

For a more complete understanding of the invention, reference is made to the detailed description taken in connection with the accompanying drawing, wherein the single figure shows 40 a more or less diagrammatic layout of the carburizing apparatus as a whole.

1 indicates a carburizing retort in a furnace 2 having a heating chamber 3 into which a plurality of burners 4 fire for heating the articles 45 in the retort to carburizing temperature. 5 indicates a pipe for supplying carburizing gas to the retort and 6 a vent through which spent gases leave the retort.

10 indicates an upright tubular charcoal retort 50 in a heating chamber 11 into which a plurality of burners 12 fire for heating the charcoal 13 in the retort to incandescence. Ordinarily the temperature in the heating chamber 11 will be maintained at approximately 1600—1800° F. The 55 retort extends through the roof 14 of the heat-

ing chamber and has a charcoal hopper 15 at its upper end, the top of the hopper being normally sealed by a removable cover 16. The gases produced in the retort pass therefrom by way of a pipe 17 shown as within the retort adjacent its 5 upper end. The pipe extends out of the retort above the roof 14 of the heating chamber and connects with a suction pump 18, the discharge side of which delivers to the pipe 5 leading to the carburizing retort 1. The hydrocarbon gas 10 is delivered to the lower end of the charcoal retort by a pipe 19 having a control valve 20.

The lower end of the retort 10 rests on a base 21 which constitutes the bottom of the heating 15 chamber 11. This base has a vertical chamber 22, the top of which is in open communication with the lower end of the retort and the column of charcoal in the retort extends down into said chamber. The lower end of the chamber 20 has a downwardly extending chute 23 which dips into an ash pan 24 adapted to contain a sealing liquid, such as water, for sealing off the lower 25 end of the chute. Ashes resulting from the operation of the gas producer are raked out of the pan as circumstances require.

25 indicates a pipe for supplying air to the chamber 22 for burning with the charcoal therein, the gases of combustion flowing upwardly into the retort 10 for further reaction therein. It is preferred that some fuel gas be admixed with the air whereby to reduce the consumption of the charcoal and to furnish gases of combustion that will react with the incandescent charcoal to produce carbon monoxide. It will be understood 30 that the reaction which takes place in the chamber 22 is exothermic whereas that which takes place in the retort 10 is endothermic.

As already stated, the heating chamber 11 will be maintained at a temperature of approximately 1600—1800° F. The reason for withdrawing the 40 gases from the retort at a point below the roof 14 of the heating chamber is to prevent the freshly formed carbon monoxide from reacting with relatively cool charcoal to the production of CO<sub>2</sub>. By flowing the hydrocarbon gas into the retort 45 10, its composition is so changed that the gases coming from the retort may be used without further treatment for carburizing articles in the carburizing retort 1. In this connection it should be stated that the gases coming from the charcoal retort have a dew point below 25° F. and, therefore, need not be dehydrated before delivering to the carburizing retort 1.

As an example of the kind of gas obtained when operating in the manner described, the fol- 50 55

lowing is cited: When 20 cubic feet of propane per hour was flowed into the retort 10 and the total amount of gas coming from the retort was 1100 cubic feet per hour, the resulting gas analyzed approximately as follows, namely: 29% CO; 0.1% CO<sub>2</sub>; 5% CH<sub>4</sub>; 15% H<sub>2</sub>; the balance being nitrogen and the dew point of the gases being below 25° F.

For the purposes of comparison, the kind of 10 gas obtained when no hydrocarbon was flowed into the retort the following is cited: 31% CO; 0.1% CO<sub>2</sub>; 1% CH<sub>4</sub>; 11% H<sub>2</sub>; the balance being nitrogen and the dew point of the gases being less than 25° F. The important differences between 15 the two kinds of gases as regards carburizing operation is the difference in methane content.

The kind of hydrocarbon gas that is flowed into the retort 10 is of more or less secondary importance, since in any event it will be broken 20 down in contact with the incandescent charcoal and yield methane which is the gas that is desired. Thus natural gas that is not pure methane may advantageously be flowed through the retort for the removal of impurities. However, it 25 is with the treatment of the higher hydrocarbons like butane and propane and mixtures of these containing propylene or butylene that the invention has special utility since it is with the higher hydrocarbons that trouble is encountered 30 when they are simply added to a weak carburiz-

ing gas such as charcoal gas to form a stronger carburizing gas.

What I claim is:

1. That method of utilizing a hydrocarbon gas to produce a carburizing gas for carburizing steel 5 articles which comprises first reacting said hydrocarbon gas with incandescent charcoal, admixing the gaseous products of such reaction with a diluent comprising carbon monoxide, and then utilizing the resulting mixture of gases as an atmosphere for said articles.

2. That method of utilizing a hydrocarbon gas to produce a carburizing gas for carburizing steel 10 articles which comprises first reacting said hydrocarbon gas with incandescent charcoal, admixing the gaseous products of such reaction with charcoal gas, and then utilizing the resulting mixture as an atmosphere for said articles.

3. That method of utilizing a hydrocarbon gas to produce a carburizing gas for carburizing steel 15 articles which comprises first reacting said hydrocarbon gas with incandescent charcoal in a retort, admixing with the gaseous products of such reaction while in said retort a diluent comprising carbon monoxide, and then withdrawing 20 the resulting mixture of gases from said retort and utilizing the same as an atmosphere for said articles.

FRANKLIN D. WIDNER. 30